

Aug. 25, 1925.

1,550,718

S. M. UDALE

PISTON RING MOLD

Filed March 14, 1923



INVENTOR.  
*Stanley M. Udale*  
BY

ATTORNEY.

Patented Aug. 25, 1925.

1,550,718

# UNITED STATES PATENT OFFICE.

STANLEY M. UDALE, OF DETROIT, MICHIGAN, ASSIGNOR TO EARL HOLLEY, OF DETROIT, MICHIGAN.

## PISTON-RING MOLD.

Application filed March 14, 1923. Serial No. 625,070.

To all whom it may concern:

Be it known that I, STANLEY M. UDALE, a citizen of the United States, residing at 893 Lothrop Ave., Detroit, in the county of 5 Wayne and State of Michigan, have invented certain new and useful Improvements in Piston-Ring Molds, of which the following is a specification.

This invention relates to piston ring 10 molds and specifically to an improved mold and core adapted to produce cast rings at a minimum cost and of uniform quality.

In the manufacture of cast iron piston 15 rings it is extremely desirable to obtain the finest possible granulation of the graphitic carbon combined with uniformity of distribution. The co-efficient of friction, resistance to wear, elasticity and resistance to shock are all factors which render piston 20 rings suitable for the severe uses to which they are put in internal combustion engines and the like, and these factors are determined by the uniform distribution of the graphitic carbon.

25 The figure shows in cross sectional elevation the mold with core and rings in place.

The mold consists of two matching hollow molds A and B inclosing a baked dry sand core C which may be provided with a 30 central conical sprue or entrance D. A plurality of horizontal gates E radiate from this central sprue D to each of the grooves F in the core C. These grooves F are uniformly spaced in the circumference 35 of the core C, except in the middle where a gap G is left.

In the middle of the core C a pair of knock-outs H and J are provided which contact with the core at the gap G referred 40 to. The outside surface of the dry sand core C, against which the piston rings are cast in the grooves F, is protected by a coating preferably of magnesium oxide, as set forth in the copending application of 45 D. H. Meloche, Serial No. 548,475, filed 31 March 1922. The powdered magnesium oxide is mixed with water and is applied with a brush or air spray, gluten being used as a binder and is dissolved in the water 50 for that purpose. The core is of course dried after being coated. This coating prevents sand being carried by the iron into the grooves where it would interfere with the subsequent machining.

55 The particular coating which has been

found best for lining the iron molds has been found to be powdered fire clay suspended in water in which water glass is dissolved to act as a binder, as set forth in the co-pending application of Daniel H. 60 Meloche, Serial No. 581,239, filed 11 August 1922. The finely ground fire clay is mixed with an equal weight of a 10% solution of sodium silicate in water. This mixture is applied with a paint brush or air 65 spray onto the heated surface of the mold, which is repeatedly heated during the painting operation so as to render the coating adherent.

A thick pulverent coating of lampblack 70 is super-imposed on the coating of soluble silicate as described in the co-pending application of D. H. Meloche, Serial No. 579,927, filed 5 August 1922.

The molds are heated to between 650° 75 and 1150° F. before the iron is poured in, the iron being considerably above 2200° F. The casting is ejected whilst it is still above its critical temperature at 1450° F. The iron poured consists of a mixture suitable 80 for piston rings, that is to say it consists of #1 foundry pig mixed with a small percentage (10%) of high grade low carbon steel scrap. The silicon content is sufficiently high (2.25%) to ensure that the major portion of the carbon content is instantaneously precipitated and uniformly distributed as fine particles of graphitic carbon throughout the ferrite mass.

85 The above process corresponds to that described in the application to D. H. Meloche, Serial No. 622,675, filed 3 March, 1923, and the product corresponds to the application of D. H. Meloche, Serial No. 618,715, filed 12 February 1923, which is a continuation 90 of Serial No. 559,463, filed 8 May 1922 by the same inventor.

A strainer core K may be placed in the entrance to the sprue D to prevent any dirt 95 being carried into the mold.

A conical re-entrant shoulder L is provided in the mold with a corresponding shoulder on the core C to prevent the ferrostatic head of the iron within the sprue D causing the core to float up in the mold 105 during the pouring operation.

110 By providing a plurality of gates E leading from the sprue D to the grooves F I ensure that the molten iron is fed to each ring groove simultaneously and at a plu-

2. rality of different points equally spaced around the circumference and so obtain uniformity throughout each ring and between all the rings.

3. The refractory fire clay coating on the molds A and B, with the pulverent coating of lampblack, render the annealing of the rings unnecessary. The rings are therefore ready for machining immediately they are

10 cast and cleaned.

When a larger ring than 6" is required a plurality of sprues will be required, each sprue feeding one sector of the circumference of each ring so as to still further increase the number of gates feeding each ring. Such an arrangement will shorten the length of the gates E so that quite large rings could be cast with comparatively short gates.

15 20 What I claim is:

1. A mold adapted for the production of individually cast piston rings, comprising a cylindrical core having a vertical axis, a plurality of circumferential grooves in said core, a substantially vertical sprue passage 25 located in the upper part of said core, a plurality of gates leading from said sprue to said grooves, a pair of metal molds enclosing said core.

2. A mold adapted for the production of 30 individually cast piston rings, comprising a cylindrical core having a vertical axis, a plurality of circumferential grooves in said core, a substantially vertical sprue passage 35 located in the upper part of said core, a plurality of gates leading from said sprue to said grooves, a mold enclosing said core.

In testimony whereof I affix my signature.

STANLEY M. UDALE.